

1

2,944,021

## MARINE DIESEL LUBRICANT

Clifford J. Ulzheimer, Woodbury Heights, and John C. Zimmer, Union, N.J., assignors to Socony Mobil Oil Company, Inc., a corporation of New York

No Drawing. Filed Jan. 25, 1956, Ser. No. 561,344

2 Claims. (Cl. 252—33.4)

This invention relates to lubricants for diesel engines. It is more particularly concerned with lubricants for marine diesels in which sour fuel oils are used as fuels.

As is well known to those familiar with the art, many types of large marine diesel engines are lubricated by injecting small amounts of a lubricant into the cylinder during each cycle. Such engines do not have conventional crank case type of lubrication wherein the continuous, copious lubrication of the pistons and cylinder walls is effected. As is further known, many of these engines burn fuels usually of the No. 6 Bunker fuel type that contain relatively large amounts of sulfur and other corrosive materials. As a result, when these oils are burned in the cylinder, there are formed quantities of corrosive acidic compound, such as sulfuric acid, sulfurous acid, etc. The presence of these materials is detrimental to the operational life of the engine because corrosion is increased and also because the presence of large amounts of strong acid promotes deposit formation and induces greater wear of the piston and of the cylinder walls.

Accordingly, it will be appreciated that it would be highly advantageous to neutralize the acidic sulfur compounds and to eliminate the corrosive effects thereof so that engine life can be prolonged. It is to be noted that the use of conventional high detergency lubricating oils has not proved to be wholly effective. Indeed, in the cases where such oils may be effective, it has been necessary to use such high concentrations of detergents that the overall operation is uneconomical.

It has now been found that corrosion and wear in the operation of marine diesels can be reduced effectively and economically. It has now been discovered that the effects of harmful deposits in marine diesels can be overcome by lubricating the engines with a novel emulsion type lubricant that tends to neutralize acidic corrosive materials and to remove them from the combustion section of the engine.

Accordingly, it is an object of this invention to reduce corrosion in marine diesel operation. Another object is to provide a lubricant that will satisfactorily neutralize acidic corrosive combustion products and remove them from the cylinder. A more specific object is to provide an emulsion type lubricant that will overcome the harmful effects of corrosive agents while still maintaining effective lubrication of a marine diesel. Other objects and advantages of this invention will become apparent to those skilled in the art from the following detailed description.

In general, the present invention provides an emulsion type lubricant for marine diesels which comprises, by weight of the lubricant, between about 10 percent and about 50 percent water (preferably between about 10 and about 35 percent), between about 80 percent and about 45 percent mineral lubricating oil (preferably between about 80 and about 55 percent), between about 1 percent and about 5 percent alkali-metal hydroxide, the amount thereof being sufficient to effect a total Base Number in the lubricant of between about 10 and about

2

100, between about 1 percent and about 10 percent oil-soluble detergent and between about 3 percent and about 10 percent of an emulsifier that effects water-in-oil type emulsion.

5 The lubricants of this invention are prepared by dissolving an alkali-metal hydroxide in the water and the oil soluble detergent in the mineral lubricating oil. The aqueous and the oil solution are then emulsified by the addition of a suitable water-in-oil type emulsifying agent 10 by any conventional means. Thus, for example, the emulsion can be produced by agitation in any suitable homogenizing equipment, such as a Manton-Gaulin Homogenizer, a Stratco Contactor, or in a mechanically agitated, heated blending kettle.

15 The basic materials that are dissolved in the aqueous phase of the lubricant are the alkali metal hydroxides. In general, lithium hydroxide is preferred because of the lower molecular weight. However, sodium and potassium hydroxides are effective. The amount of alkali metal compound used will be between about one percent and about 5 percent, by weight of finished lubricant. Sufficient must be used, however, to produce a total Base Number (ASTM Test D664-54) of 10-100, preferably 10-50.

20

25 The mineral oil content of the lubricant of this invention will be the usual hydrocarbon lubricant utilizable for the lubrication of heavy machinery. Generally, this lubricating oil will be a petroleum hydrocarbon fraction or a blend of two or more fractions, of the No. 20 to

30 No. 50 SAE grade. In terms of Saybolt Universal viscosity, the mineral oil will have a viscosity of 45-100

seconds at 210° F., and preferably of 75-80 seconds at

210° F. The mineral lubricating oil can be obtained from any crude source or sources. It is especially pre-

35 ferred, however, to use a naphthenic oil, such as one obtained from a coastal crude.

The detergents that are dissolved or dispersed in the oil phase are, in general, the additives used in detergent motor oils. Usually they are polyvalent metal salts of

40 organic acids. Non-limiting examples include petroleum sulfonates, such as barium "mahogany" sulfonate, magnesium petroleum sulfonate, etc.; wax-substituted aryl sulfonates, such as barium di-wax benzene sulfonate, calcium tri-wax benzene sulfonate, barium wax naphthalene sulfonate, etc.; sulfurized or unsulfurized phenates and carboxylates, such as sulfurized calcium phenate, barium wax phenate, magnesium wax benzene carboxylate, etc. The detergents are not exactly equivalent and the selection of a particular detergent will depend 45 upon the emulsifier used. Some detergents will destroy the emulsion characteristics with some emulsifiers, but will be found to be compatible with others.

As has been mentioned hereinbefore, the oil phase and the aqueous phase are maintained in a stable water-in-oil emulsion by means of a suitable emulsifying agent.

50 In general the emulsifying agent can be a sulfonate, such as sodium mahogany sulfonate, ammonium naphthalene sulfonate, etc.; esters of high molecular weight acids obtained by controlled oxidation of petroleum fractions; fatty acid soaps, such as sodium oleate, "red oil" soaps, potassium stearate, ammonium linoleate, etc.; and the like. The preferred type of emulsifiers are a non-metallic material, such as the ammonium soaps and the oxidized

55 petroleum acid esters. It is to be understood, however, that emulsifying agents are not equally effective and that the effectiveness of a given emulsifying agent will be affected by the types and the concentrations of the various other ingredients of the lubricant. The effectiveness 60 of an emulsifying agent in any given formulation can readily be determined by those skilled in the art by subjecting a sample to an oven storage test at 130-135°

F. A stable emulsion lubricant will not separate after 16 hours of storage.

The relative concentrations of the ingredients of the lubricant in this invention can vary over fairly wide ranges. Generally, the amount of basic material used will be at least enough to effectively reduce the acidity of the corrosive combustion products. The amount of detergent used must be at least enough to provide effective detergent action, while the amount of emulsifier will be sufficient to maintain a stable water-in-oil emulsion.

It has been found that the ranges within which the concentration of the various components of the emulsion type lubricant of this invention can be varied are within the following ranges, based upon the weight of the finished lubricant:

|                         | Percent |
|-------------------------|---------|
| Basic compound          | 1-5     |
| Detergent               | 1-10    |
| Emulsifier              | 3-10    |
| Mineral lubricating oil | 80-45   |
| Water                   | 10-50   |

It is to be understood that the lubricant of this invention can contain other additives for the purpose of imparting other properties to the lubricant. Thus, for example, there can be added anti-rust agents, E.P. (extreme pressure) agents, antioxidants, and the like.

#### Example

Into a blending kettle equipped with a mechanical agitator, were placed 5 parts, by weight, of an emulsifier (Alox 1657), 2 parts, by weight, of a detergent (Lubrizol 1220), and 60 parts, by weight, of a mineral lubricating oil. The emulsifier, Alox 1657, is a mixture of esters of high molecular weight acids obtained by controlled oxidation of petroleum oil, that is sold by the Alox Corp., Niagara Falls, New York. "Alox 1657" has the following typical properties:

|                             |                |
|-----------------------------|----------------|
| Acid number                 | Max. of 4.0.   |
| Saponification number       | 30-40.         |
| Color                       | Dark brown.    |
| Ash—ASTM-D-482-46           | 0.07%.         |
| Melting point—ASTM-D-127-49 | 120° F.        |
| Viscosity @ 210° F.         | 220-240 S.U.S. |
| Specific gravity @ 146° F.  | 0.874.         |
| Average weight per gallon   | 7.3 lbs.       |
| Flash (O.C.)                | 450° F. (min.) |
| Fire (O.C.)                 | 540° F. (min.) |

Further details as to the nature and properties of this material are available in Alox Technical Data Sheet on Alox L-1657, April 1952. The detergent, Lubrizol 1220, is a calcium petroleum sulfonate sold by the Lubrizol Corp., Cleveland, Ohio. The mineral lubricating oil is a blend containing 38 volume percent of a solvent refined coastal oil having a Saybolt viscosity of 150 seconds at 210° F. and 62 volume percent of a solvent refined coastal oil having a Saybolt viscosity of 55 seconds at 210° F. This blend has an A.P.I. gravity of 24 degrees and a Saybolt viscosity of about 75 seconds at 210° F. The mixture of oil detergent and emulsifier was heated with agitation at 130° F. until the solution was complete. It was then cooled to 100-110° F. In a separate vessel was dissolved three parts by weight of lithium hydroxide monohydrate in thirty parts by weight of water.

This solution was slowly added to the oil blend in the blending kettle. Continuous vigorous agitation was maintained throughout the blending period. After all the lithium hydroxide solution had been added vigorous agitation was continued for an additional 15 minutes in order to obtain the emulsion. This emulsion was then passed through a Manton-Gaulin Homogenizer operated at 3000 to 3500 pounds p.s.i.g. Continuous agitation was maintained in the blending kettle while the emulsion was being transferred to the homogenizer.

The water-in-oil emulsion lubricant thus produced had the following physical characteristics:

|   |                          |       |
|---|--------------------------|-------|
| 4 | A.P.I. gravity           | 17.6  |
|   | SUS viscosity at 100° F. | 2,247 |
|   | SUS viscosity at 130° F. | 868   |
|   | SUS viscosity at 210° F. | 168.5 |
| 5 | Viscosity index          | 112   |
|   | Total base No.           | 40    |

This lubricant was placed aboard a commercial motor vessel that was powered with an 8 cylinder, 2 cycle, double acting Gotaverkin diesel engine. This ship was operated continuously for seven days coastal voyage. During this time, two cylinders were lubricated with the emulsion lubricant of this example and six cylinders were lubricated with a standard marine lubricant of the mineral oil type. This oil was a blend of 57 volume percent solvent refined coastal oil of 150 seconds Saybolt at 210° F. and 43 volume percent solvent refined coastal oil of 55 seconds Saybolt at 210° F. It had an A.P.I. gravity of 24° and a Saybolt viscosity at 210° F. of 97 seconds. At the completion of the run, it was found that the cylinders lubricated with the emulsion type lubricant operated freely and had received adequate lubrication.

This application is a continuation-in-part of copending application Serial No. 541,847, filed October 20, 1955, and now abandoned.

Although the present invention has been described with preferred embodiments, it is to be understood that modifications and variations may be resorted to, without departing from the spirit and scope of this invention, as those skilled in the art will readily understand. Such variations and modifications are considered to be within the purview and scope of the appended claims.

We claim:

1. An emulsion lubricant for marine diesels which consists of, by weight of the lubricant, between about 10 percent and about 35 percent water, between about 80 percent and about 55 percent mineral lubricating oil having a Saybolt Universal viscosity of between about 75 seconds and about 80 seconds measured at 210° F., between about 1 percent and about 5 percent alkali-metal hydroxide, said alkali-metal hydroxide being present in the water phase of said lubricant, the amount thereof being sufficient to effect a total base number in the lubricant of between about 10 and about 50, between about 1 percent and about 10 percent oil soluble polyvalent metal sulfonate and between about 3 percent and about 10 percent esters of high molecular weight acids obtained by controlled oxidation of petroleum oil.

2. An emulsion lubricant for marine diesels which consists of, by weight of the lubricant, about 30 percent water, about 60 percent naphthenic mineral lubricating oil having a Saybolt Universal viscosity of about 75 seconds measured at 210° F., about 5 percent lithium hydroxide, said lithium hydroxide being present in the water phase of said lubricant, about 2 percent calcium petroleum sulfonate, and about 3 percent esters of high molecular weight acids obtained by controlled oxidation of petroleum oil; said oil lubricant having a total base number of about 40.

#### References Cited in the file of this patent

#### UNITED STATES PATENTS

|           |                      |               |
|-----------|----------------------|---------------|
| 2,079,051 | Sullivan et al.      | May 4, 1937   |
| 2,320,263 | Carlson et al.       | May 25, 1943  |
| 2,671,758 | Vinograd et al.      | Mar. 9, 1954  |
| 2,727,005 | McKinley et al.      | Dec. 13, 1955 |
| 2,744,870 | Stillebroer et al.   | May 8, 1956   |
| 2,820,007 | Van Der Minne et al. | Jan. 14, 1958 |

#### OTHER REFERENCES

"Alox Corporation Technical Data Sheet" on Alox L-1657, April 1952, pub. by Alox Corp., 70 Pine Street N. Y. N. Y., page 1.